

## UNITED STATES PATENT OFFICE

2,126,737

MANUFACTURE OF ARTICLES FROM POW-  
DERED MATERIALSGregory J. Comstock, Fairfield, Conn., assignor  
to Handy & Harman, Bridgeport, Conn., a cor-  
poration of New YorkNo Drawing. Application August 10, 1935,  
Serial No. 35,631

8 Claims. (CL. 75—22)

This invention relates generally to the manufacture of articles from powdered metals and more particularly to the manufacture of articles such as silverware, jewelry and objects of art 5 from precious metals or mixtures of precious metals with base metals. The invention is particularly described in connection with the use of powdered precious metals such as silver, gold, platinum, iridium, palladium and the like. 10 Among the base metals which may be used in conjunction with the precious metals are copper, nickel, zinc, antimony, cobalt, molybdenum, tungsten, titanium, tantalum, iron, and alloys of these metals.

15 Powdered metals are used for a wide variety of purposes, among which may be mentioned the production of porous material for use as bearings, and the production of cutting tools where the powdered materials employed are generally 20 the refractory metals or their carbides. The present invention relates to the production of solid, that is, non-porous, articles as contrasted with those suitable for bearings. By the term "non-porous", I mean compositions which are 25 relatively free from pores as compared with those compositions suitable for bearings and which are usually made porous intentionally so as to hold a lubricant.

The "non-porous" compositions of the present 30 invention are those which are sufficiently dense so that they do not work materially differently from the melted and cast alloys and have strengths and other properties not materially different from cast alloys. The metals which I employ are the precious metals either alone or 35 in conjunction with smaller amounts of base metals as contrasted with compositions containing the refractory metals such as tungsten or tantalum or their carbides in large amount, which 40 compositions are employed for the production of cutting tools, drawing dies and the like. By the use of powdered metals, articles can be made of various compositions which would not be possible to make by a melting and casting process due to the fact that in such melting and casting processes the composition in many cases is limited by the tendency of the metals employed to alloy with each other in different proportions.

The present invention is applicable to the production 45 of ornamental objects having designs thereon made from powdered metal. In one method of making such objects a presintered base of powdered copper, for example, may be stamped with a rubber stamp, moistened with an adhesive such as glycerine or gum tragacanth

so as to form the desired design on the presintered base. Lines, lettering or designs may be applied in this way in a very simple manner. Powdered silver is then sprinkled over the presintered base and the excess powder which does not stick to the adhesive is shaken off and the base with the powdered silver adhering thereto in the desired design is placed in a mold and hot pressed. In the hot pressing operation, a highly polished metal plunger thinly coated with graphite or lamp black is used to prevent the plunger sticking to the applied powder. The pressure employed in the hot pressing step may be, for example, 2000-4000#/sq. in. in order to consolidate the powder and densify the presintered base. 15

Powdered metal may be applied to a cast and rolled base rather than to a presintered base by the method just described of applying powdered metal to an adhesive applied in a design to a base, and the base with the applied powder may 20 then be subject to hot pressing as previously described. A design of copper inlaid on a rolled sheet of sterling silver has been successfully made according to this process.

For purposes of illustration I have described 25 the invention particularly with reference to the use of silver and copper. It will be understood, however, that other combinations of powdered metals may be employed and that the invention 30 may be otherwise embodied or practiced within the scope of the following claims.

I claim:

1. The method of forming an inlaid article, which comprises forming a sintered body from powdered material, applying powdered material 35 to the sintered body by the use of an adhesive, and sintering the powdered material and consolidating it with the sintered body by the application of heat and pressure.

2. The method of forming an inlaid article, 40 which comprises forming a sintered body from powdered material by the simultaneous application of heat and pressure, applying powdered material to the sintered body by the use of an adhesive, and sintering the powdered material and 45 consolidating it with the sintered body by the application of heat and pressure.

3. The method of forming an inlaid article, which comprises forming a sintered body from powdered material by the simultaneous application of heat and pressure, applying powdered material to the sintered body by the use of an adhesive, and sintering the powdered material and 50 consolidating it with the sintered body by the simultaneous application of heat and pressure.

greater than the heat and pressure employed in forming the sintered body to which the powdered material was applied.

4. The method of forming an inlaid article, which comprises simultaneously heating and 5 pressing powdered material to form a sintered body, applying an adhesive to the sintered body in the desired design, applying powdered material to the sintered body and shaking off the excess which does not adhere to the adhesive, and sub- 10 jecting the sintered body with the powdered material adhering thereto in the desired design to the simultaneous application of heat and pressure greater than the heat and pressure employed in forming the sintered body.
- 15 5. The method of forming an inlaid article, which comprises applying powdered material in a design to a base by the use of an adhesive, and subjecting the base and applied powdered material to simultaneous heat and pressure suf- 20 ficient to sinter and consolidate the design with the base.

6. The method of forming an inlaid article, which comprises applying powdered precious metal in a design to a base by the use of an adhesive, and subjecting the base and applied powdered precious metal to simultaneous heat and pressure sufficient to sinter and consolidate the design with the base. 5

7. The method of forming an inlaid article, which comprises applying powdered material in a design to a cast and rolled base by the use of 10 an adhesive, and subjecting the base and applied powdered material to simultaneous heat and pressure sufficient to sinter and consolidate the design with the base.

8. The method of forming an inlaid article, 15 which comprises applying powdered precious metal in a design to a cast and rolled base by the use of an adhesive, and subjecting the base and applied powdered precious metal to simultaneous heat and pressure sufficient to sinter and consolidate 20 the design with the base.

GREGORY J. COMSTOCK.